

Sept. 3, 1968

M. W. SHAFER

3,399,957

MAGNETIC MATERIALS AND PROCESS OF PREPARATION

Filed Jan. 16, 1968



INVENTOR  
MERRILL W. SHAFER

BY *Hansel L. McGee*

ATTORNEY

3,399,957  
MAGNETIC MATERIALS AND PROCESS  
OF PREPARATION

Merrill W. Shafer, Yorktown Heights, N.Y., assignor to International Business Machines Corporation, Armonk, N.Y., a corporation of New York  
Continuation-in-part of application Ser. No. 374,321, June 11, 1964. This application Jan. 16, 1968, Ser. No. 698,350

4 Claims. (Cl. 23—52)

## ABSTRACT OF THE DISCLOSURE

New divalent europium magnetic materials, having the formula  $Eu_xAl_2O_{3+x}$  where  $x=1, 3$  or  $5$ , have been prepared. A mixture of divalent europium oxide and aluminum oxide is heated in a nonoxidizing atmosphere and cooled. The compounds are transparent crystalline materials which may be used in magneto-optical devices.

This application is a continuation-in-part of my pending application, Ser. No. 374,321 filed on June 11, 1964, now abandoned and entitled, Magnetic Materials and Process of Preparation.

## Background of the invention

Field of the invention.—This invention relates to new europium aluminate magnetic materials and, in particular, to those magnetic materials having the formula  $Eu_xAl_2O_{3+x}$  where  $x=1, 3$  or  $5$  and their preparation. In single crystal form, these new magnetic materials are transparent and thus can be utilized in magneto-optical devices.

## Description of the prior art

Magnetic materials generally fall into two classes, those which exhibit cooperative magnetism, and those which do not. Those with the cooperative magnetic effect are the ferromagnetic, ferrimagnetic and anti-ferromagnetic materials. The great majority of the ferromagnetic materials are metals and good electrical conductors, hence, opaque materials. The ferrimagnetic materials can have a range of resistivities, but their conduction bands are partially filled and also are opaque for all practical purposes. Although the antiferromagnetic materials can have unfilled conduction bands, their net magnetic moments are small and consequently have little practical use.

The existence of insulating ferromagnetic or ferrimagnetic materials are rare since they would require that the conduction band be unfilled and still exhibit a positive interaction involving unpaired electrons. Examples of these materials would be  $CrBr_3$ ,  $Na_4Fe_3F_{14}$  and the following silicates of europium,  $Eu_2SiO_4$ ,  $Eu_3SiO_5$ . On the other hand, the yttrium iron garnets, e.g.,  $Y_3Fe_5O_{12}$  and rare earth iron garnets only partially fill these requirements, since they are only transparent in very thin sections.

It is well known that when a light is passed through a magnetic material in which there are unpaired electrons, there will be an interaction and the light will be rotated in a manner which is dependent on the alignment and the number of unpaired electron spins of the material (i.e., the Faraday effect). This Faraday effect is usually defined in terms of the Verdet's constant which is the observed rotation in minutes per gauss per centimeter thickness. This is also true in the case of paramagnetic materials as well as in the case of ferromagnetic and ferrimagnetic materials. Thus, the greater the number of unpaired electrons and their ability to align in a magnetic field, the greater will be the specific rotation of the light that the material can transmit (i.e., the specific rotation

is directly proportional to the magnetic susceptibility of the material).

## Summary of the invention

A group of europium aluminate magnetic materials has been prepared, the members of which have unpaired electrons and are transparent in relatively thick layers in the visible and near visible spectrum (i.e., wavelengths greater than about 4500 Å.). These materials have the formula  $Eu_xAl_2O_{3+x}$  where  $x=1, 3$  or  $5$ . Those europium aluminates where  $x=3$  or  $5$  exhibit a high saturation magnetization. The europium aluminate where  $x=1$  is paramagnetic. All the europium aluminates are chemically stable under ordinary conditions and optically transparent in a single crystal form.

It is an object of the invention to prepare europium aluminate magnetic materials.

It is a further object of the invention to prepare europium aluminate magnetic materials having the formula  $Eu_xAl_2O_{3+x}$  where  $x=1, 3$  or  $5$  and which are transparent.

Another object of the invention is to prepare a paramagnetic material having the formula  $EuAl_2O_4$ .

Still another object of the invention is to prepare a ferromagnetic material having the formula  $Eu_3Al_2O_6$ .

A still further object of the invention is to prepare a ferromagnetic material having the formula  $Eu_5Al_2O_8$ .

Further, another object of the invention is a magneto-optical device utilizing a crystal of  $Eu_xAl_2O_{3+x}$  where  $x=1, 3$  and  $5$ .

The foregoing and other objects, features and advantages of the invention will be apparent from the following more particular description of a preferred embodiment of the invention, as illustrated in the accompanying drawing.

The drawing is a diagrammatic showing of a magneto-optical device utilizing a europium aluminate crystal of the present invention.

In the magneto-optical device shown diagrammatically in the drawing, a single crystal (or crystal section) 1 of a ferro- or paramagnetic europium aluminate of the present invention is mounted between spaced crossed polarizing filters (i.e., polarizer 2 and analyzer 3). The crystal is placed in a magnetic field (e.g., that produced by an electromagnet 4 or by Helmholtz coils). A light source 5 and a photosensitive cell 6 are so disposed that the light to which the photosensitive cell is exposed is that which originates at the light source and passes successively through polarizer 2, crystal 1 and analyzer 3. Since the degree of rotation of the plane of polarized light passing through the paramagnetic crystal is dependent upon the magnetic field, the amount and orientation of light originating in the light source and passing through the polarizer and analyzer and crystal to the photosensitive cell can be varied by varying the strength of the magnetic field of the magnet. In the ferromagnetic region, above magnetic saturation, the rotation is independent of the applied magnetic field and the maximum rotation can be obtained.

All these europium aluminate materials have high Verdet's constants even at room temperature because of their high magnetic susceptibility and high degree of transparency. As a result of this high Verdet's constant, all these europium aluminate materials can be used in magneto-optical devices such as laser beam modulators, light switches, etc. The compounds  $Eu_3Al_2O_6$  and  $Eu_5Al_2O_8$  exhibit a very large Faraday rotation at helium temperature. In addition, the new ferromagnetic materials, which are insulators, have properties which find application in memory elements, transformer cores, or in any device where high resistivity, low coercive force material is desired at low temperatures.

Table I gives the magnetization data showing magnetic susceptibility versus temperature in degree Kelvin for the three europium aluminates. The saturation magnetization and Curie temperature data are shown in the right column. All measurements were made using standard techniques.

5

TABLE I

| Temp.<br>(° K.)                    | Magnetic<br>Susceptibility<br>( $X_{-6}$ )<br>(10 c.g.s.) | Magnetic Saturation Properties |
|------------------------------------|-----------------------------------------------------------|--------------------------------|
| $\text{EuAl}_2\text{O}_4$          |                                                           |                                |
| 300                                | 81                                                        |                                |
| 250                                | 100                                                       |                                |
| 200                                | 120                                                       |                                |
| 150                                | 168                                                       |                                |
| 100                                | 245                                                       |                                |
| 50                                 | 500                                                       |                                |
| 42                                 | 5,720                                                     |                                |
| $\text{Eu}_3\text{Al}_2\text{O}_6$ |                                                           |                                |
| 300                                | 120                                                       |                                |
| 250                                | 142                                                       |                                |
| 200                                | 183                                                       |                                |
| 150                                | 250                                                       |                                |
| 100                                | 380                                                       |                                |
| 50                                 | 800                                                       |                                |
| $\text{Eu}_5\text{Al}_2\text{O}_8$ |                                                           |                                |
| 300                                | 87                                                        |                                |
| 250                                | 100                                                       |                                |
| 200                                | 126                                                       |                                |
| 150                                | 165                                                       |                                |
| 100                                | 250                                                       |                                |
| 50                                 | 500                                                       |                                |

The  $\text{Eu}_x\text{Al}_2\text{O}_{3+x}$  (where  $x=1, 3$  and  $5$ ) magnetic materials are prepared by reacting intimate mixtures of  $\text{EuO}$  or  $\text{EuCO}_3$  or  $\text{Eu(OH)}_2$  and  $\text{Al}_2\text{O}_3$  at elevated temperatures between  $800^\circ$ – $1600^\circ$  C. under nonoxidizing conditions such as an oxygen free vacuum or any condition in which there is an absence of oxygen, such as argon, nitrogen, etc., or under reducing atmosphere containing large percentages of hydrogen, e.g., nitrogen with hydrogen added (1–100 percent hydrogen).  $\text{CO}_2$  with approximately 20–80 percent hydrogen, argon containing 1–100 percent hydrogen and pure hydrogen.

The following specific examples represent embodiments of the invention and, more particularly, disclose the preparation of the europium aluminate magnetic materials.

#### Example I— $\text{Eu}_3\text{Al}_2\text{O}_6$

50.4 grams of  $\text{EuO}$  are intimately mixed with 10.2 grams of  $\text{Al}_2\text{O}_3$ . This mixture is then placed in an iridium crucible. The crucible was raised to a temperature greater than  $1000^\circ$  C. in a pure hydrogen atmosphere and held at that temperature for 36 hours. The crucible was then cooled to room temperature at a rate of  $50^\circ$  C. per minute. The resultant product  $\text{Eu}_3\text{Al}_2\text{O}_6$  is a ruby red polycrystalline powder with a Curie temperature of  $10^\circ$  K. The product is X-rayed. The pattern is shown below.

| Line | $d$  | $I/I_0$ |
|------|------|---------|
| 1    | 5.57 | 10      |
| 2    | 3.94 | 30      |
| 3    | 3.54 | 5       |
| 4    | 2.70 | 100     |
| 5    | 2.74 | 10      |
| 6    | 2.61 | 10      |
| 7    | 2.28 | 15      |
| 8    | 2.27 | 10      |
| 9    | 2.14 | 05      |
| 10   | 2.11 | 10      |
| 11   | 1.97 | 20      |
| 12   | 1.85 | 10      |
| 13   | 1.76 | 05      |
| 14   | 1.60 | 20      |
| 15   | 1.61 | 20      |

An elemental analysis of the product gave the following results:

|                        | Theory<br>(percent) | Found<br>(percent) |
|------------------------|---------------------|--------------------|
| Total Eu.....          | 75.3                | 75.6±0.5           |
| Total Al.....          | 8.9                 | 8.6±0.2            |
| Eu <sup>++</sup> ..... |                     | 74.6±0.5           |

#### Example II— $\text{EuAl}_2\text{O}_4$

10 16.8 grams of  $\text{EuO}$  are intimately mixed with 10.2 grams of  $\text{Al}_2\text{O}_3$ . This mixture is then placed in a platinum crucible. The crucible is placed in an oven and the temperature is raised to  $1200^\circ$  C. in a pure argon atmosphere and held at that temperature for 25 hours. The crucible was then cooled to room temperature at a rate of  $50^\circ$  C. per minute. The resultant product  $\text{EuAl}_2\text{O}_4$  is a light red powder which is paramagnetic down to  $1.8^\circ$  K. The product is X-rayed. The pattern is shown below.

20

| Line | $d$   | $I/I_0$ |
|------|-------|---------|
| 1    | 6.09  | 5       |
| 2    | 5.16  | 5       |
| 3    | 4.44  | 100     |
| 4    | 4.41  | 30      |
| 5    | 4.22  | 10      |
| 6    | 3.90  | 5       |
| 7    | 3.14  | 85      |
| 8    | 3.05  | 85      |
| 9    | 2.988 | 75      |
| 10   | 2.57  | 25      |
| 11   | 2.556 | 60      |
| 12   | 2.47  | 5       |
| 13   | 2.42  | 5       |
| 14   | 2.21  | 15      |
| 15   | 1.95  | 10      |
| 16   | 1.93  | 10      |
| 17   | 1.86  | 15      |

25

35 An elemental analysis of the product gave the following results:

|                        | Theory<br>(percent) | Found<br>(percent) |
|------------------------|---------------------|--------------------|
| Total Eu.....          | 56.4                | 55.9±0.5           |
| Total Al.....          | 20.0                | 20.1±0.2           |
| Eu <sup>++</sup> ..... |                     | 55.2±0.5           |

#### Example III— $\text{Eu}_5\text{Al}_2\text{O}_8$

40 45 84 grams of  $\text{EuO}$  and 10.2 grams of  $\text{Al}_2\text{O}_3$  are intimately mixed. This mixture is placed in a carbon crucible and the crucible is placed in an oven. The temperature was raised to  $1600^\circ$  C. in a pure nitrogen atmosphere and held at that temperature for 12 hours. The resultant product  $\text{Eu}_5\text{Al}_2\text{O}_8$  is a powder with a dark red color and a 50 Curie temperature of  $6^\circ$  K. The product is X-rayed. The pattern is shown below.

50

| Line | $d$  | $I/I_0$ |
|------|------|---------|
| 1    | 5.49 | 10      |
| 2    | 5.07 | 10      |
| 3    | 3.61 | 40      |
| 4    | 2.90 | 48      |
| 5    | 2.87 | 100     |
| 6    | 2.86 | 95      |
| 7    | 2.77 | 10      |
| 8    | 2.74 | 35      |
| 9    | 2.33 | 30      |
| 10   | 2.33 | 50      |
| 11   | 2.30 | 15      |
| 12   | 2.13 | 10      |
| 13   | 1.80 | 20      |
| 14   | 1.77 | 10      |
| 15   | 1.68 | 20      |
| 16   | 1.61 | 10      |
| 17   | 1.53 | 05      |

60

65 An elemental analysis of the product gave the following results:

|                        | Theory<br>(percent) | Found<br>(percent) |
|------------------------|---------------------|--------------------|
| Total Eu.....          | 80.6                | 79.4±0.5           |
| Total Al.....          | 5.7                 | 6.1±0.2            |
| Eu <sup>++</sup> ..... |                     | 79.6±0.5           |

70

75

The devices of the present invention have been described as made up essentially of a crystal containing  $\text{Eu}_2\text{Al}_2\text{O}_{3+x}$  which is placed in a magnetic field and associated optical instrumentation in order to utilize the Faraday effect. These devices may be manufactured according to the techniques known in the art for the manufacture of analogous devices embodying other crystal bodies. The best results are obtained when the specific rotation of the light passing through the crystal varies linearly with the applied magnetic field.

However, the maximum rotation obtainable for this material can be obtained when operated in the ferromagnetic state, i.e., below their Curie temperature 10° K. for  $\text{Eu}_3\text{Al}_2\text{O}_6$  and 6° K. for  $\text{Eu}_5\text{Al}_2\text{O}_8$ .

The new europium aluminates of the invention have the formula  $\text{Eu}_x\text{Al}_2\text{O}_{3+x}$  where  $x=1, 3$  and  $5$ . These aluminates are transparent and thus are used in magneto-optical devices.

While the invention has been particularly shown and described with reference to a preferred embodiment thereof, it will be understood by those skilled in the art that various changes in form and details may be made

therein without departing from the spirit and scope of the invention.

What is claimed is:

1. A compound having the formula  $\text{Eu}_x\text{Al}_2\text{O}_{3+x}$  where  $x=1, 3$  and  $5$ .
2. The compound  $\text{EuAl}_2\text{O}_4$ .
3. The compound  $\text{Eu}_3\text{Al}_2\text{O}_6$ .
4. The compound  $\text{Eu}_5\text{Al}_2\text{O}_8$ .

10 **References Cited**

UNITED STATES PATENTS

- |           |         |              |       |         |
|-----------|---------|--------------|-------|---------|
| 3,282,856 | 11/1966 | Borchardt    | ----- | 23—50 X |
| 3,294,701 | 12/1966 | Vogel et al. | ----- | 23—50 X |

15 **OTHER REFERENCES**

Warsaw et al.: "Inorganic Chemistry", vol. 1, August 1962, pp. 719—720.

20 OSCAR R. VERTIZ, *Primary Examiner*.

H. T. CARTER, *Assistant Examiner*.